# EUROPEAN PATENT SPECIFICATION

(11) **EP 0 381 886 B1**
(45) Date of publication and mention of the grant of the patent: **08.12.1993**
(21) Application number: 89309041.5
(22) Date of filing: 06.09.1989
(51) Int. Cl.: E01F 9/08

(54) **Surface marker strip**
Oberflächenmarkierungsstreifen
Bande de marquage sur des surfaces

(30) Priority: 10.02.1989 US 309312
(43) Date of publication of application: 16.08.1990
(73) Proprietor: BRITELINE CORPORATION, West Roxbury Massachusetts (US)
(72) Inventor: Wyckoff, Charles W., Needham Massachusetts (US)
(74) Representative: Allsop, John Rowland

(56) References cited:
- DE-A- 2 544 059
- DE-B- 2 208 983
- US-A- 3 399 607
- US-A- 3 587 415
- US-A- 4 117 192
- US-A- 4 388 359
- US-A- 4 490 432
- US-A- 4 681 401

## Description

The present invention relates to surface marker strips as for roadways, pavements and other surfaces, being more particularly directed to methods of providing better roadway-adhering and longer-life properties to such marker strips, and to marker strips or tapes with preformed ridges adhered to the roadways and the like of vastly improved integrity and life that, by reflection and/or retroreflection from the ridges, enable enhanced visibility, especially upon illumination by the headlights of approaching vehicles.

A paramount problem with preformed plastic pavement marker strips of the prior art is that of providing satisfactory adherence to the road surface under the constant heavy pounding of motor vehicle traffic. Unless the pavement marker has a deformable layer of elastomeric material which lacks memory positioned between the marker and the road surface, good adhesion will not always be achieved. This layer must deform readily and flow without memory into the irregular surface contours of the pavement. The deformability and ability to cold flow permits the absorption of the energy of vehicle tire impacts which would otherwise violently dislodge the pavement marker as the impact energy is dissipated. With an elastic material, adhesion to the road surface is weakened when the road is wet because the stretch-return action of such a memory material causes a pumping action to occur in which water-bearing dirt is forced between the material and the road surface. Dirt then becomes deposited between the adhesive material and the road surface and ultimately destroys the adhesive properties holding the pavement marker to the road.

While for some applications, techniques for adhesion of the type employed with marker strips of my earlier U.S. Letters Patent Nos. 3,920,346; 4,040,760; 4,069,787; 4,236,788 and 4,681,401 involving a thick mastic, provided a measure of the deformability and cold flow characteristics discussed above, for extensive use and under severe traffic and temperature varying circumstances, however, this technique proved at best to be only a compromise. Additionally, the mastic adhesive proved difficult to apply to the product in an economical manner. During extensive heat of summer, the adhesive had a tendency to flow readily as it became warm, with the result that the pavement-marker would creep or move with very heavy traffic. Sometimes the extremely low temperatures of winter, moreover, would reduce the bonding force between the adhesive and the pavement marker with the disasterous result of removal by snowplow action.

This problem of adequately securing a preformed plastic pavement-marker tape to the road surface was also recognized and partially solved in prior are U.S. Letters Patent Nos. 3,399,607; 3,587,415 and 4,117,192 and others. The techniques proposed in these patents involved base materials which exhibit desirable characteristics of deformability and lack of memory or cold flow which will provide conformability to the road surface and will absorb the shock energy of vehicular traffic. While useful for preformed flat surface pavement-marker tapes, however, such techniques do not adequately solve the problem for strips or tapes having preformed ridges such as those disclosed in my said earlier patents cited above. Because such prior art material has no memory and exhibits cold flow characteristics, any protruberance such as a ridge or wedge on the surface very quickly disappears when impacted by vehicular traffic so that the ridges flatten out and lose shape under the pressure of the vehicle tires. This, of course, defeats the primary purpose of high visibility of the protruberances or ridges at low veiwing angles. If the ridges were comprised of a harder or more rigid material such as, for example, polyvinyl choride or epoxy or some other rigid or semi-rigid material, they would soon be engulfed by the non-memory cold flow characteristic of the base material under the pressure of the traversing traffic. Once depressed into the base material, the ridges would no longer protrude above a film of rain water and would thus be useless as high visibility ridges for wet night visibility.

As disclosed in U.S. Letters Patent No. 4,490,432 which incorporates the teachings of Patent No. 4,388,359, an attempt was made to solve this problem by including reinforcing fibers with the mix of the non-memory cold-flowing elastomeric base material. It was hoped that the fiber would offer sufficient stiffness to overcome the problem of losing the protruberances upon impact of high volume vehicular traffic. This, however, has not proven to be a completely successful solution; and in a short time, the protruberances become, in practice, flattened into the base material where they lose their function and utility.

Underlying the present invention, on the other hand, is the discovery that a combined-layered non-vulcanized and vulcanizable rubber sheeting can admirably provide a superior solution to the above-mentioned problems. The conformability and shock energy absorbing features of a non-vulcanized elastomeric rubber sheeting when combined with a vulcanizable elastomeric rubber serving as the top portion of the tape or strip and in which the protruberances or ridges are formed enables the attainment of the novel results herein. After vulcanizing the top layer containing the ridges, the ridges can be stretched or flattened or otherwise depressed or deformed by vehicular traffic, but, because of their memory characteristics, will be restored to their original shape after cessation of said traffic. While the elastic property of the vulcanized top portion comprising the ridge structure contains sufficient memory to permit such restoration of shape, such is not enough to inhibit deformability of the soft elastomeric bottom portion which conforms to the road surface and which, with its non-memory property, readily absorbs the shock energy of the wheel impacts of the vehicular traffic.

An object of the invention, accordingly, is to provide a new and improved marker strip or tape for roadways and the like that is not subject to the previously described short-comings of prior devices but that, through a layered combination of a non-vulcanized lower rubber-like surface that conformably adheres to the roadway and an upper vulcanized rubber-like surface containing the marker ridges provides long-lasting adhesion and integrity of the ridges during use.

Other and further objects will be explained hereinafter and are more particularly delineated in the appended claims.

According to one aspect of the invention there is provided a marker strip for a roadway, comprising a rubber-like sheet having a bottom layer and surface for adhesive attachment to the roadway, and an upper layer with a reflective upper surface from which incident light from a vehicle travelling along the roadway may be reflected to indicate the roadway direction characterised in that the upper layer is cross-link vulcanized so as to provide said upper layer with memory characteristics to enable restoration of depression of the upper layer caused by vehicle wheels travelling thereover while the bottom layer remains unvulcanized with cold-flow characteristics and conformably adheres to the roadway. The invention will now be described with reference to the accompanying drawings,
Figure 1 of which is a cross-section through an single ply rubber sheeting prior to embossing the protruberances or ridges;
Figure 2 is a cross-section through a single ply rubber sheeting after embossing the protruberances or ridges;
Figure 3 is a cross-section through a double ply rubber sheeting prior to embossing the protruberances or ridges;
Figure 4 is a cross-section through a double ply rubber sheeting after embossing the protruberances or ridges; and
Figures 5 and 6 are cross-sections similar to Figures 2 and 4 after the protruberances have been formed and showing retro-reflection glass microsphere distribution on the surfaces.

Referring to the drawings, the base material 1 of the marker strip or tape is shown as comprised of a non-vulcanized rubber mixture in sheet form which lacks memory and is easily deformed because it is soft and exhibits cold flow characteristics. It is comprised of a rubber polymer such as acrylonitrile-butadiene in a non- vulcanized state. In addition reinforcing fibers, a pigment, and other processing aids are also included. An example of a typical formulation is listed in Table I in which the reinforcing fiber is given as wood pulp-like cellulose fibers. Other types of fibers including thermoplastic reinforcing fibers may be used without seriously degrading the deformability characteristic of the sheeting. In accordance with the invention, the bottom portion or layer of this material is left in this un-vulcanized cold-flow non-memory condition, and is attached by adhesive 6 (Figures 5 and 6) along the bottom surface to the roadway R. The top portion of the rubber sheeting material comprising the marker strip, however, is to be vulcanized to provide it with memory characteristics. Toward this end, the top layer may be treated as by a shallow layer of peroxide material 1′ which penetrates the rubber sheeting to a limited depth depicted by the speckled area of Figures 1 and 2. Because of the presence of peroxide or equivalent treatment, this region of the rubber sheeting can be readily cross-linked or vulcanized by the addition of heat. Prior to the heat, it has the same characteristics as the remainder of the sheet; i.e. it is soft, easily deformed and lacks memory. As illustrated in Figure 2, the sheet of Figure 1 has been embossed in the top surface with protruding wedges or ridges 3 and then heat is applied immediately thereafter in order to cross-link or vulcanize and harden this ridged top layer that had been permeated with peroxide, imparting to the ridges a permanent memory such that they can maintain shape with cold flow after vehicular depression, while the bottom of the sheeting 1 remains unvulcanized (not cross-linked) and thus deformable and memory-free to provide the necessary shock energy absorption of vehicular traffic and with conformability, to assist the adhesion in securing the marker to the road surface R. The protruding ridges or wedges 3 may be in the form of transversely extending parallel rows, successively longitudinally spaced along the strip, and may be segmented into ridge or wedge blocks, if desired, preferably with a trapezoidal crosssection providing inclined or near-vertical front and rear surfaces 1′′ for reflecting incident low-angle headlight illumination as described in said patents.

Figures 3 and 4 illustrate another method of accomplishing the same effect. In this case, the rubber sheeting base material consists of a two-ply laminate comprising a vulcanizable upper layer 2 laminated on top of a non-vulcanizable rubber sheeting layer 1. Layer 2 may contain the same ingredients as layer 1 in addition to vulcanizing agents, such as sulfur (Table II) or other compounds which react with the rubber to cross-link or vulcanize it to completion after the protruberances 3, Figure 4, have been formed. Once vulcanized, the protruberances or ridges will maintain their shapes because the vulcanization process provides the material with a memory and a degree of surface hardness.

In Figure 5, the top-embossed surface of Figure 4 has a retro-reflecting bead-bonding layer 4 covering the entire surface. This layer may be any suitable bead bonding layer such as a vinyl acetate copolymer, a polyurethane, an epoxy or any material which will satisfactorily bond the glass retroreflective microspheres 5 to the structure, curing during the curing of the upper layer of the strip. The bead bonding layer 4 can be applied to the surface either prior to or after the ridges are embossed or otherwise formed. The coating of glass microspheres or beads 5 is applied to this layer 4 prior to solidification of the layer. After vulcanization of the top ridged layer, the beads become secured in a partially embedded manner therein with the beads partially exposed including especially on the inclined or near-vertical front and rear surfaces 1′′ of the ridges or protruberances facing traffic.

As shown in the cross-section of Figure 6, the glass microspheres 7 are embedded in the cross-linked top portion of the rubber sheeting of Figure 2. This can be accomplished prior to embossing or during the embossing process itself. The glass microspheres 7 are only partially embedded on the near-vertical or inclined faces of the ridges 3, whereas those shown typically at 8 are fully embedded during the embossment. In order to promote adhesion of these microspheres to the product, it has been found that silane is helpful either incorporated with the base material or as a coating on the microspheres or both. The adhesive layer 6, shown in Figures 5 and 6, bonds the marker to the road surface R and should exert as little influence as possible on the conformability characteristics of the product to insure good adhesion to the road surface.

The marker strips or tapes of the invention may be formed by the following illustrative methods of construction which provide the ability to maintain the ridged shape and still permit road surface conformability to assist in good adhesion thereto.

### EXAMPLE 1

The ingredients listed in Table 1 below, were compounded using a lab roll mill and calender to form a sheet approximately 0.13cm (0.050) inch thick by 10cm (4 inches) wide by several tens of cms (feet) long. A squeegee was then used to apply a liquid layer of methanol and t-butyl perbenzoate onto the surface of the sheeting where a limited penetration of the surface with resulting peroxide occured. After drying with warm air for 30 seconds, the sheeting was then passed between a nip roller and a patterned embossing drum to impress a ridged pattern 3 into the top surface of the sheeting. The embossed material was then heated at 180°C (350°F) for 3 minutes during which time the upper layer 1' (Figure 2) of the rubber sheeting impregnated with the peroxide became cross-linked. The surface durometer was measured at 65-70, whereas before treatment with the peroxide it was only 40.

The embossed strip containing the ridged pattern was then positioned beneath a flat sheet of metal and the wheel of a 1 1/2 ton pick-up truck which was allowed to stand over this strip for 10 minutes, depressing the ridges. Inspection of the sample showed that the ridges had flattened to approximately 10% of their normal height. After a 10-minute waiting period, it was observed that the strip showed full recovery of the ridges and restoration to original shape. A similar test but without application of the peroxide failed to recover at all when subjected to the wheel loading for as short a time as 15 seconds.

Similar shape recovery or restoration from depression has been observed with actual vehicular travel as well.

**TABLE I**

| Material | Parts by Weight |
|---|---|
| Acrylonitrile butadiene non-crosslinked elastomer ("Hycar 1022" supplied by B.F. Goodrich) | 100 |
| Chlorinated paraffin ("Chlorowax 70-S" supplied by Diamond Shamrock) | 70 |
| Chlorinated paraffin ("Chlorowax 40") | 5 |
| Reinforcing wood-pulp-like cellulose fibers¹ | 120 |
| Pigment² | 130 |
| Glass microspheres (0.003 inch average diameter with a refractive index of 1.5) | 200 |
| Silica filler ("Hysil 233" supplied by PPG Industries) | 20 |

| | |
|---|---|
| 1 ("Interfibe" supplied by Sullivan Chemical) | |
| 2 Titanium dioxide ("Tronox CR800" supplied by Kerr-McGee Chemical) | |

**TABLE II**

| Material | Parts by Weight |
|---|---|
| Precipitated sulfur | 3 |

### EXAMPLE 2

The ingredients in TABLE 1 were compounded into sheet form as in EXAMPLE 1 to form two separate sheets 1 and 2 (Figure 3). The sheet 1 was calendered to a thickness of 0.10cm (0.040 inch). The layer 2, after the addition of precipitated sulfur in the amount of 3% total weight of rubber, was calendered to produce a 0.05cm (0.020) inch thick sheet. The sheets 1 and 2 were then laminated together and impressed with a ridged pattern 3 and heated at 180°C (350°F) for 9 minutes during which time the sulfur reacted with the rubber to effect vulcanization of the upper embossed layer 2 (Figure 4). As in EXAMPLE 1, the strip was subjected to the truck tire weight for 10 minutes and reacted in a similar manner to the previous test, recovering fully after a 10 minute waiting period.

### EXAMPLE 3

The procedure of EXAMPLE 2 was repeated except that a layer of isocyanate polyol liquid polyurethane such as sold under the trademark "Amershield" of Ameron Company, was applied on top of the sulfur-containing layer and a layer of glass microspheres 5 (Figure 5) was applied to the liquid polyurethane layer 4 prior to embossing the ridged pattern. After the polyurethane was dry to the touch, the material was embossed and then subjected to 180°C (350°F) heat for 9 minutes. The truck tire test results were similar to those of EXAMPLE 1 and the glass microspheres were noted to be unchanged and firmly anchored.

### EXAMPLE 4

The procedure of EXAMPLE 2 was repeated except that, prior to embossing, the sulfur-containing top surface 2 was given an overcoat of a 20% solution of Dow Corning Z6040 "Silane" in methanol, followed by application of glass microspheres. The treated sheet was then subjected to 180°C (350°F) for 30 seconds and then embossed with a ridged pattern. The embossing procedure caused the beads 7 to be partially embedded on the near vertical faces and almost entirely embedded on the horizontal surfaces (Figure 6). After embossing, the sheet was heated at 180°C (350°F) for 9 minutes to complete the vulcanization of the sulfur containing layer. The truck tire test results were similar to those of EXAMPLE 1 and the glass microspheres were observed to be unchanged and securely anchored to the vulcanized rubber.

Further modifications will also occur to those skilled in this art and such are considered to fall within the spirit and scope of the invention as defined in the appended claims.

## Claims

1. A marker strip for a roadway, comprising a rubber-like sheet having a bottom layer (1) and surface for adhesive attachment to the roadway, and an upper layer (1', 2) with a reflective upper surface (1'',5) from which incident light from a vehicle travelling along the roadway may be reflected to indicate the roadway direction characterised in that the upper layer (1',2) is cross-link vulcanized so as to provide said upper layer (1',2) with memory characteristics to enable restoration of depression of the upper layer (1',2) caused by vehicle wheels travelling thereover while the bottom layer (1) remains unvulcanized with cold-flow characteristics and conformably adheres to the roadway.

2. A roadway marker strip as claimed in claim 1 and in which said reflective surface is formed by successively positioned retro-reflective bead protuberances (5) partially embedded in said upper layer (1',2).

3. A roadway marker strip as claimed in claim 1 and in which said upper layer (1',2) has wedge or ridge protuberances (3), at least the forward and rearward sides of the protuberances (3) having reflective beads (5) partially embedded therein.

4. A roadway marker strip as claimed in any preceding claim and in which the upper layer (1',2) and bottom layer (1) are the parts of an integral sheet.

5. A roadway marker strip as claimed in any one of claims 1 to 3 and in which the upper and bottom layers are a pair of laminated sheets (1,2) with only the upper layer (2) vulcanized.

6. A roadway marker strip as claimed in any preceding claim and in which the bottom layer (1) is provided with adhesive (6) along its exposed surface for contacting the roadway.

7. A method of preparing a roadway marker strip comprising providing a rubber-like sheet having a bottom layer (1) and surface for adhesive attachment to the roadway and an upper layer (1',2) with a reflective surface (1'',5) from which incident light from a vehicle travelling along the roadway may be reflected, characterised by treating the upper layer (1') and surface to condition the same for heat treatment, and cross-link vulcanizing the upper layer (1',2) and surface under the heat treatment while maintaining cold-flow characteristics in the bottom layer (1) and surface of the sheet to enable restoration of depression of the upper layer (1',2) and surface under vehicle traffic accompanied by conformance of the lower layer (1) to the roadway.

8. A method as claimed in claim 7 and in which successively positioned retro-reflective bead protuberances (5) are partially embedded in said upper layer to form said reflective surface before said cross-link vulcanizing under heat treatment.

9. A method as claimed in claim 7 and in which a formation of wedge or ridge protuberaces (3) is provided in the upper layer (1',2), and partially embedding retro-reflective beads (5) at least in the forward and rearward sides of the protuberances (3).

10. A method as claimed in claims 8 or 9 and in which said beads (5) are applied in a binder (4) that cures with the said upper layer (1',2) and surface.

11. A method as claimed in any one of claims 7 to 10 and in which said heat treatment is with sulphur, with said upper layer being a separate sheet (2) that is vulcanized and laminated to a separate cold-flow bottom sheet to form said bottom layer (1).

## Patentansprüche

1. Ein Markierungsstreifen für eine Fahrbahn, bestehend aus einem gummiartigen Flachmaterial mit einer Bodenschicht und einer Oberfläche für eine klebende Befestigung an der Fahrbahn, sowie aus einer oberen Schicht (1', 2) mit einer reflektierenden Oberseite (1'', 5), von der auftreffendes Licht eines sich entlang der Fahrbahn bewegenden Fahrzeugs reflektiert werden kann, um die Richtung der Fahrbahn anzuzeigen, **dadurch gekennzeichnet,** daß die obere Schicht (1', 2) für eine Vernetzung vulkanisiert ist, um so der oberen Schicht (1', 2) eine Memory-Charakteristik zu verleihen und die Behebung von Eindrücken in der oberen Schicht (1', 2) zu ermöglichen, welche durch sich darüber bewegende Fahrzeugräder bedingt sind, während die Bodenschicht (1) unvulkanisiert mit Kaltfluß-Charakteristiken verbleibt und gleichförmig an der Fahrbahn haftet.

2. Ein Fahrbahn-Markierungsstreifen nach Anspruch 1, bei dem die erwähnte reflektiertende Oberseite durch sukzessiv oder aufeinanderfolgend positionierte reflektierende perlen- oder kugelartige Vorsprünge (5) gebildet ist, die in der oberen Schicht (1', 2) teilweise eingebettet sind.

3. Ein Fahrbahn-Markierungsstreifen nach Anspruch 1, bei dem die erwähnte obere Schicht leisten- bzw. rippenartige oder rückenartige Erhebungen (3) aufweist, wobei wenigstens die Vorder- und Rückseiten der Erhebungen die dort teilweise eingebetteten reflektierenden Kugeln oder Perlen (5) aufweisen.

4. Ein Fahrbahn-Markierungsstreifen nach einem der vorhergehenden Ansprüche, bei dem die obere Schicht (1', 2) und die Bodenschicht Teil eines einstückigen Flachmaterials sind.

5. Ein Fahrbahn-Markierungsstreifen nach einem der Ansprüche 1 - 3, bei dem die obere Schicht und die Bodenschicht ein Paar von laminierten Schichten (1, 2) bilden, wobei lediglich die obere Schicht (2) vulkanisiert ist.

6. Ein Fahrbahn-Markierungsstreifen nach einem der vorhergehenden Ansprüche, bei dem die Bodenschicht (1) an ihrer für die Berührung mit der Fahrbahn freiliegenden Oberfläche mit einem Kleber (6) versehen ist.

7. Ein Verfahren zum Herstellen eines Fahrbahn-Markierungsstreifens, bei welchem ein gummigartiges flaches Material bereitgestellt wird, welches eine Bodenschicht (1) und eine Oberfläche für eine Klebe-Befestigung an der Fahrbahn sowie eine obere Schicht (1', 2) mit einer reflektierenden Oberfläche (1'', 5) besitzt, von der auftreffendes Licht von einem Fahrzeug, welches sich entlang der Fahrbahn bewegt, reflektiert werden kann, gekennzeichnet durch Behandlung der oberen Schicht (1') und der Oberfläche, um diese für eine Wärmebehandlung zu konditionieren, sowie durch Vernetzungs-Vulkanisierung der oberen Schicht (1', 2) und Oberseite durch die Hitzebehandlung, während die Kaltfluß-Charakteristiken in der Bodenschicht (1) und der Oberfläche des flachen Materials erhalten bleiben, um die Behebung von Eindrücken in der oberen Schicht (1', 2) sowie in der Oberfläche zu ermöglichen, die vom Fahrzeugverkehr herrühren, und zwar verbunden mit einer Anpassung der unteren Schicht an die Fahrbahn.

8. Ein Verfahren nach Anspruch 7, bei dem wieder reflektierende perlen- oder kugelförmige Vorsprünge aufeinanderfolgend in der oberen Schicht eingebettet werden, um die erwähnte reflektierende Oberfläche zu bilden, und zwar vor der Vernetzungsvulkanisation durch Wärmebehandlung.

9. Ein Verfahren nach Anspruch 7, bei dem leisten- oder dachartige Vorsprünge (3) in der oberen Schicht (1', 2) vorgesehen und die wieder reflektierenden Kugeln oder Perlen (5) wenigstens an den Vorder- und Rückseiten der Vorsprünge eingebettet werden.

10. Ein Verfahren nach den Ansprüchen 8 oder 9, bei dem die erwähnten Perlen oder Kugeln (5) in einem Binder (5) vorgesehen werden, der mit der erwähnten oberen Schicht (1', 2) und der Oberseite aushärtet.

11. Ein Verfahren nach einem der Ansprüche 7 - 10, bei dem die Wärmebehandlung mit Schwefel erfolgt, wobei die erwähnte obere Schicht eine separate Schicht (2) ist, die vulkanisiert und mit einem separaten Bodenflachmaterial zur Bildung der erwähnten Bodenschicht (1) laminiert bzw. verbunden wird.

## Revendications

1. Bande de signalisation pour une chaussée, comprenant une feuille semblable à du caoutchouc ayant une couche inférieure (1) et une surface de fixation par collage sur la chaussée, et une couche supérieure (1', 2) avec une surface supérieure réfléchissante (1'', 5) sur laquelle la lumière incidente d'un véhicule se déplaçant le long de la chaussée peut se réfléchir afin d'indiquer l'orientation de la chaussée, caractérisée en ce que la couche supérieure (1', 2) est vulcanisée par réticulation afin de former ladite couche supérieure (1', 2) avec des caractéristiques de mémoire qui permettent de reformer l'affaissement de la couche supérieure (1', 2) provoqué par les roues du véhicule se déplaçant dessus tandis que la couche inférieure (1) reste non vulcanisée avec des carctéristiques de fluage à froid et adhère à la chaussée en s'y conformant.

2. Bande de signalisation pour chaussée selon la revendication 1, dans laquelle ladite surface réfléchissante est formée en plaçant successivement des bossages (5) en forme de perles réfléchissantes partiellement enrobés dans ladite couche supérieure (1', 2).

3. Bande de signalisation pour chaussée selon la revendication 1, dans laquelle ladite couche supérieure (1', 2) porte des bossages (3) en forme d'arêtes ou de nervures, les côtés avant et arrière au moins des bossages (3) ayant des perles réfléchissantes (5) partiellement enrobées à l'intérieur.

4. Bande de signalisation pour chaussée selon l'une quelconque des revendications précédentes, dans laquelle la couche supérieure (1', 2) et la couche inférieure (1) sont les parties de la feuille intégrée.

5. Bande de signalisation pour chaussée selon l'une quelconque des revendications 1 à 3, dans laquelle les couches supérieure et inférieure constituent une paire de feuilles lamifiées (1, 2) dont seule la couche supérieure (2) est vulcanisée.

6. Bande de signalisation pour chaussée selon l'une quelconque des revendications précédentes, dans laquelle la couche inférieure (1) est couverte d'un adhésif (6) sur sa surface apparente afin de venir en contact avec la chaussée.

7. Procédé de préparation d'une bande de signalisation pour chaussée comprenant la formation d'une feuille analogue à du caoutchouc ayant une couche inférieure (1) et une surface destinée à être fixée par collage sur la chaussée et une couche supérieure (1', 2) avec une surface réfléchissante (1'', 5) sur laquelle la lumière incidente d'un véhicule se déplaçant le long de la chaussée peut se réfléchir, caractérisé par le traitement de la couche supérieure (1') et de la surface pour les préparer à un traitement thermique, et la vulcanisation par réticulation de la couche supérieure (1', 2) et de la surface sous l'effet du traitement thermique tout en gardant les caractéristiques de fluage à froid de la couche inférieure (1) et de la surface de la feuille pour permettre de rétablir l'affaissement de la couche supérieure (1', 2) et de la surface sous l'effet de la circulation des véhicules en même temps que la conformité de la couche inférieure (1) avec la chaussée.

8. Procédé selon la revendication 7, dans lequel des bossages en forme de perles réfléchissantes (5) placés successivement sont partiellement enrobés dans ladite couche supérieure pour former ladite surface réfléchissante avant ladite vulcanisation par réticulation sous l'effet du traitement thermique.

9. Procédé selon la revendication 7, dans lequel la formation de bossages (3) en forme d'arêtes ou de nervures est prévue dans la couche supérieure (1', 2) ainsi que l'enrobage partiel de perles réfléchissantes (5) au moins dans les faces avant et arrière des bossages (3).

10. Procédé selon la revendication 8 ou 9, dans lequel lesdites perles (5) sont appliquées dans un liant (4) qui durcit en même temps que ladite couche (1', 2) et surface supérieure.

11. Procédé selon l'une quelconque des revendications 7 à 10, dans lequel ledit traitement thermique se fait avec du soufre, ladite couche supérieure étant une feuilles distincte (2) qui est vulcanisée et lamifiée sur une feuille inférieure distincte de fluage à froid pour forer ladite couche inférieure (1).
